



US005141542A

**United States Patent** [19]

Fangeat et al.

[11] **Patent Number:** **5,141,542**[45] **Date of Patent:** \* Aug. 25, 1992[54] **FIRE RESISTANT TEXTILE YARN AND USE THEREOF**[75] Inventors: **Roland Fangeat, Vert Le Petit; Pierre Christ, Epinal; Alain Choserot, Golbey, all of France**[73] Assignee: **Filature de la Gosse S.A., Golbex, France**

[\*] Notice: The portion of the term of this patent subsequent to Nov. 6, 2007 has been disclaimed.

[21] Appl. No.: **446,097**[22] Filed: **Dec. 5, 1989****Related U.S. Application Data**

[63] Continuation-in-part of Ser. No. 159,574, filed as PCT/EP/8700293, Jun. 4, 1986, Pat. No. 4,967,548.

[30] **Foreign Application Priority Data**

Jun. 4, 1986 [FR] France ..... 86 08024

[51] **Int. Cl.**<sup>5</sup> ..... **D02G 3/02; D02G 3/12; D02G 3/18; D02G 3/38**[52] **U.S. Cl.** ..... **57/224; 57/229; 428/364; 428/373; 428/377; 428/392; 428/393; 428/395**[58] **Field of Search** ..... **428/364, 365, 392, 379, 428/395, 393; 57/210, 229**

[56]

**References Cited****U.S. PATENT DOCUMENTS**

|           |         |                      |         |
|-----------|---------|----------------------|---------|
| 2,932,587 | 4/1960  | Labino .....         | 428/392 |
| 3,729,920 | 5/1973  | Sayers et al. ....   | 57/229  |
| 3,913,309 | 10/1975 | Chiarotto .....      | 57/229  |
| 4,015,038 | 3/1977  | Romanski et al. .... | 428/255 |
| 4,381,639 | 5/1983  | Kress .....          | 57/229  |
| 4,383,403 | 5/1983  | Nakayama et al. .... | 428/377 |
| 4,500,593 | 2/1985  | Weber .....          | 57/229  |
| 4,670,327 | 6/1987  | Weber .....          | 428/377 |
| 4,838,017 | 6/1989  | Kolmes et al. ....   | 57/210  |
| 4,967,548 | 11/1990 | Fangeat et al. ....  | 428/364 |

**OTHER PUBLICATIONS**

Modern Textile Dictionary p. 935 Table III, Conversion of English Cotton Count Into Rounded Tex Number.

Kirk-Othmer, vol. 3, "Aramid Fibers" pp. 213-215, 224.

*Primary Examiner*—Patrick J. Ryan

*Assistant Examiner*—J. M. Gray

*Attorney, Agent, or Firm*—Cushman, Darby & Cushman

[57] **ABSTRACT**

Disclosed herein is a fire-resistant textile yarn comprising a core formed from an inorganic filament surrounded by fibres formed entirely or in part from aramid resin. Also disclosed is a fire-resistant textile yarn comprising a core formed from a ply yarn comprising double-threaded - multi-glass filaments, the core being surrounded by fibres formed entirely or in part from aramid resin.

**5 Claims, No Drawings**

## FIRE RESISTANT TEXTILE YARN AND USE THEREOF

This is a continuation-in-part of U.S. application Ser. No. 07/159,574 filed as PCT/EP8700293, Jun. 2, 1987, now U.S. Pat. No. 4,967,548.

### BACKGROUND OF THE INVENTION

#### 1 Field of the Invention

In one embodiment, the present invention relates to a fire-resistant textile yarn comprising an inorganic filament core surrounded by fibers formed at least in part from aramid resin. In a second embodiment, the present invention relates to a fire-resistant textile yarn comprising a core formed from a ply yarn comprising double-threaded-multi-glass filaments, the core being surrounded by fibers formed at least in part by aramid resin.

2. Background Information aramid fibers to produce 20 yarn for making a fire-resistant material. The aramid fibers are similar in appearance to polyamide 6—6 fibers and are resistant to bending and equivalent abrasion. However, while polyamide 6—6 melts at 250° C., aramid fibers at this temperature have a resistance to rupture equivalent to 60% of their resistance at room temperature. Aramid fibers do not melt, but begin to deteriorate above 370° C.

U.S. Pat. No. 4,381,639 discloses a yarn of the type comprising a core, formed from a continuous filament comprising at least 96% SiO<sub>2</sub>, surrounded by aramid fibers, the mass ratio of fibers/core being 40:60 with a core 0.5 mm in diameter. Yarn of this type is unsuitable for making clothing fabric, but can only be used for producing protective fabric for items of safety clothing which are only to be worn for performing special tasks, for a limited period. The mass ratio of aramid fibers and the core is too low to ensure proper covering of the core. As the aramid fibers are pigmented and the filament of the core is not, this core will appear in the 40 fabric. Although poor covering of the core is acceptable for safety clothing for professional use only, this is not the case when the fabric is intended for clothing which, in addition to its fire-resistant properties, is also to comprise an item of clothing, the appearance and 45 comfort of which should be comparable to those of ordinary fabric. This is especially the case with fabrics used in making uniforms.

It is obvious that if, in the case of the type of yarn disclosed in the aforementioned document, it were desirable to increase substantially the mass ratio of aramid fibers relative to that of the core, the yarn count would at the same time be increased and would therefore become too high for making clothing fabric.

The thickness of the filament used to form the core of 55 the yarn is in particular imposed by the twisting which this filament undergoes during the operation to spin the aramid fibers around the core, twisting which a substantially finer filament would not tolerate or which would excessively weaken it.

It has likewise been proposed in U.S. Pat. No. 4,384,449 with a core made from an inorganic substance around which two aramid filaments or yarns formed from aramid fibers are wound along two counter-directional helices. Where the core is surrounded by aramid fibers the yarns are spun beforehand, so that the resulting yarn is a type of twister yarn formed about a core. The aramid fibers are therefore not spun around a

frame. It is obvious that a yarn of this type can be used to produce a protective fabric, particularly for making gloves, but would not be suitable for making clothing fabric.

It will be seen that the heat-resistant yarns proposed by the prior art can be used to manufacture protective fabrics, but could not be used to make fabrics suitable for clothing. Fabrics of this type should have, in addition to their properties for protecting against heat and 10 fire, the appearance of any other clothing fabric and adequate mechanical resistance to stress and rupture. This fabric must obviously be permeable to air and vapour to allow physiological exchanges to occur, and its surface unit weight should not be too great, but 15 should be comparable to that of normal clothing fabric.

The aim of the present invention is to propose a solution combining these different requirements.

### SUMMARY OF THE INVENTION

In one embodiment, the present invention relates to a heat-resistant textile yarn comprising an inorganic filament core surrounded by fibers formed at least in part from aramid resin, wherein the yarn count is between 30-50 tex, the mass ratio of the core is between 10% and 25%, and the aramid fibers are spun around this core without axial twisting.

In a second embodiment, the present invention relates to the use of the textile yarn of the first embodiment in making clothing fabric, wherein the warp yarn count is 30 10% to 20% lower than the weft yarn count, the inorganic filament of the warp yarn makes up 10% to 15% of the mass of the yarn count, and the inorganic filament of the weft yarn accounts for 20% to 25% of the yarn count.

In a third embodiment, the present invention is directed to a heat-resistant textile yarn comprising a core formed from a ply yarn comprising double-threaded-multi-glass filaments, the core being surrounded by fibers formed at least in part from aramid resin, wherein the yarn count is between 30 and 55 tex, the mass ratio of the core is between 10% and 26%, and the aramid fibers are spun around this core without axial twisting.

In a fourth embodiment, the present invention is directed to the use of the textile yarn of the third embodiment in making clothing fabric, wherein the warp yarn count is preferably the same as the weft yarn count.

### DETAILED DESCRIPTION OF THE INVENTION

As noted above, in one embodiment, the present invention is related to a heat-resistant textile yarn comprising an inorganic filament core surrounded by fibers formed at least in part from aramid resin, wherein the yarn count is between 30-50 tex, the mass ratio of the core is between 10% and 25%, and the aramid fibers are spun around this core without axial twisting.

In a second embodiment, the present invention relates to the use of this yarn in making clothing fabric, wherein the warp yarn count is 10% to 20% lower than 60 the weft yarn count, the inorganic filament of the warp yarn makes up 10% to 15% of the mass of the yarn count, and the inorganic filament of the weft yarn accounts for 20% to 25% of the yarn count.

In contrast to yarns with a glass core surrounded by aramid fibers or a mixture comprising at least a proportion of these fibers, spun with axial twisting of the core, for example using the open end spinning process, the present yarn is provided with a core which is not axially

twisted, which means that the proportion of core can be reduced substantially. This means that a much finer yarn can be produced in which the core has a better covering of fibers, and means that a much more flexible yarn can be produced. The finer the core, the more flexible the yarn and the easier it is to conceal it with a layer of fibers. In a fire-resistant fabric formed by a conventional yarn with a glass core, it is difficult to conceal the core completely, without making a thick yarn, the core already being relatively thick on its own. Although fabric of this type is acceptable for making work clothing, it is not so for making a uniform for example, for which the appearance should obviously not be in any way different from that of traditional fabric, even though special properties are required.

The manufacture of the present yarn with a fine non-axially twisted core, more particularly with a monofilament is achieved by what is known as the DREF process, performed by a spinning frame made by the FEHRER company. According to this process, the 20 fibers are wound around the core. Since the core is not subjected to axial twisting as in the conventional spinning process, it is therefore possible to use a glass monofilament which, for a yarn of 30 to 50 tex, makes up between 10% and 25% by weight of this yarn, i.e. a 25 filament of between approximately 50 and 80  $\mu\text{m}$ .

Two different yarns have been manufactured using this principle. The first is a yarn of 50 tex comprising a glass monofilament of 11 tex having a diameter of approximately 75  $\mu\text{m}$  surrounded by 50% Kermel  $\text{R}$  aramid fibers made by Rhone-Poulenc and 50% viscose fibers spun on a DREF 3 machine. The strength of this yarn is 10N, its coefficient of variation a % of the strength CV%R is 3.5 and its % extension is 3%.

The second of these yarns has a count of 42 tex and 35 comprises a glass monofilament of 5.5 tex having a diameter of approximately 50  $\mu\text{m}$  surrounded by fibers comprising 50% Kermel  $\text{R}$  aramid fibers made by Rhone-Poulenc and 50% viscose fibers spun on a DREF 3 machine. The strength of this yarn is 6N, its 40 coefficient of variation as a % of the strength CV%R is 3.5 and its regain is 3%.

These two yarns were used for manufacturing a herringbone twill fabric from Kermel  $\text{R}$  viscose 220 with a glass core. The thicker yarn of 50 tex with a glass core 45 of 11 tex is used as the weft yarn and appears on the reverse side of the fabric, while the finer of 42 tex with a glass core of 5.5 tex is used as the warp yarn and thus comprises the visible part of the fabric. As a result of this combination, the thicker weft yarn, provided with a 50 core having a diameter 50% greater than that of the warp yarn improves the strength of the fabric. However, even if the covering of the glass core of the weft yarn is not complete, with the herringbone twill this 55 yarn only appears on the reverse side of the fabric. Contrastingly, the finer core of the warp yarn, where it provides the yarn with lower strength, allows better covering of the glass core and appears on the visible side of the fabric.

The fabric manufactured in this way underwent a 60 number of tests carried out by the Institut Textile de France. These tests were performed in accordance with the AFNOR (French Standards Institute) standards in a normal atmosphere with relative humidity of 65% and at a temperature of 20° C. The mass of the fabric per  $\text{m}^2$  according to French standard NF G 07104 was 225 g and permeability to air in accordance with AFNOR G 07111 was tested on a TEXTTEST permeability meter.

The value is expressed in liters of air passing through 1  $\text{m}^2$  of fabric per second ( $1/\text{m}^2/\text{s}$ ) with a depression of 20 mm of water. This permeability was 458 (402-528).

Table 1 below gives the mechanical properties of the 5 fabric measured in the direction of the warp and the weft. The rupture force and the extension at rupture are measured in accordance with French standard NF 07119 on samples of 20  $\times$  5 cm using an INSTRON 1175 electronic dynamometer with a constant extension gradient. The induced rupture is measured in accordance with AFNOR G 07148 using a Lhomargy ruptumeter (high capacity active force pendulum ram impact testing machine). The behaviour during repeated folding was tested in order to determine the loss in rupture 15 strength after being folded 10,000 times using an ITF Lyon flexometer with rollers on which the sample is folded alternately in the forward direction and the reverse direction. The dynamometric measurement was taken in order to determine the loss in rupture strength after being folded 10,000 times.

TABLE 1

|                                   | Warp             | Weft             |
|-----------------------------------|------------------|------------------|
| Rupture force daN                 | 73.2 (71.4-74.4) | 86.6 (80.6-90.8) |
| % Extension at rupture            | 13.5 (13.1-13.9) | 6.9 (6.6-7.5)    |
| Induced rupture daN               | 3.6 (3.3-3.7)    | 4.6 (4.3-5.0)    |
| Behaviour during repeated folding |                  |                  |
| Normal fabric strength daN        | 73 (71.9-74.7)   | 83.4 (78.9-89.4) |
| after 10,000 folds daN            | 73.8 (71.9-75.6) | 77.2 (74.5-79.3) |
| Loss in strength                  | 0%               | 7.4%             |

This fabric also underwent inflammability tests in accordance with AFNOR standard G 07113. The table below gives the values measured using six samples, three warp and three weft:

TABLE 2

| Warp Samples | Area of the charred region $\text{cm}^2$ | Weft samples          | Area of the charred region $\text{cm}^2$ |
|--------------|------------------------------------------|-----------------------|------------------------------------------|
| 1            | 14                                       | 4                     | 10                                       |
| 2            | 13                                       | 5                     | 11                                       |
| 3            | 11                                       | 6                     | 16                                       |
| Average      | 13                                       | Average               | 12                                       |
|              |                                          | Overall average: 12.5 |                                          |

The same fabric underwent water-proofing and oil-proofing treatment using two products: a water-proofing product by Ciba-Geigy sold under the trade name of Phobotex  $\text{R}$  FTC which is a derivative of the condensation of formaldehyde and an amino 1,3,5 triazine with 1 or 2NH<sub>2</sub> groups and an oil-proofing agent by the 3M company marketed in France by Ciba-Geigy under the trade name Scotchgard  $\text{R}$  FC 232.

The Kermel viscose 220 herringbone twill lo fabric with the glass core treated in this way underwent surface wetting comparison tests in accordance with the standard NF G 07056, water penetration tests according to standard NF G 07057 and oil penetration tests according to the Scotchgard AATCC 118 method. To carry out this comparison a Kermel/Viscose 205 herringbone twill fabric was used.

The tests were performed on two samples of fabric after treatment, and on samples which had been dry cleaned in the presence of perchlorethylene without RB 65 1/10 booster for 20 minutes and dried at room temperature.

The Table below gives the results measured after the various tests. The table comprises three columns ST,

SCHMERBER and OLEO referring respectively to surface wetting by spray, penetration by water and the Scotchgard method developed by the 3M company and accepted as a universal reference; each of these three columns is subdivided into two columns EO and IN indicating respectively the measurement taken from the fabric before cleaning and from the fabric after dry cleaning in the aforementioned conditions. For the ST and OLEO tests the figures correspond to performance indices 1 to 5, the last figure indicating the best performance. With regard to the SCHMERBER test the figures indicate the height of the water column in mm to obtain fabric penetration.

TABLE 3

| ST                | SCHMER-<br>BER |    |         | OLEO    |    |    |
|-------------------|----------------|----|---------|---------|----|----|
|                   | EO             | IN | EO      | IN      | EO | IN |
| Grey/green KV 205 | 5              | 2  | 180-190 | 160-170 | 5  | 2  |
| Glass core KV 220 | 5              | 2  | 130-140 | 150-150 | 5  | 2  |

Where it is desirable for the fabric to be able to undergo thermal treatment in order, in particular, to remove harmful chemical products with which it has been impregnated, it may be advantageous to replace the glass core with a metal core in order to provide the possibility of heating by inducing an electric current in the metal core. In the case of steel for example with a 50 tex yarn, the maximum diameter of the filament would be limited to 45  $\mu\text{m}$  for a proportion by weight of 25%. 30

On the other hand, it would be possible to form filaments of B or SiC on a core of W 13  $\mu\text{m}$  in diameter on which boron is deposited by the chemical decomposition of  $\text{BCl}_3$ . The same process can be used to produce filaments of W/SiC. This information is contained in the 35 "Encyclopaedia of Chemical Technology" Kirk-Othmer, Third edition, Volume 6, page 296 (John Wiley and Sons). Given the low density of the boron or the SiC it is possible to make filaments which are stronger than steel for an equivalent cross section. In that case, and so as not to exceed the proportion of 25% for 40 yarns of 50 tex, the W/B filaments may have a maximum diameter of 75  $\mu\text{m}$  and those of W/SiC 65  $\mu\text{m}$  allowing for the tungsten core of 13  $\mu\text{m}$ . Naturally, filaments of this type allow the proportion by weight of 45 the core to be reduced relative to this maximum value whilst providing the fabric with good mechanical strength, the filaments being able to be made to the required diameter by accretion about the initial tungsten core of 13  $\mu\text{m}$ .

In a third embodiment of the present invention, which represents an improvement over the

first embodiment, a fire-resistant textile yarn comprises a core formed from a ply yarn comprising double-threaded - multi-glass filaments, the core being surrounded by fibers formed entirely or in part from aramid resin, wherein the yarn count is between 30 and 55 tex, the mass ratio of the core is between 10% and 26%, and the aramid fibers are spun without axial twisting around the core.

A fourth embodiment of the present invention is directed to a method of making a clothing fabric, which comprises weaving into the clothing fabric the yarn of the third embodiment, wherein the warp yarn count of the yarn is preferably the same as the weft yarn count.

The core yarn of the third embodiment of the present invention is thus formed from a ply yarn comprising double-threaded-multi-glass filaments, rather than the

single filament of glass of the first embodiment of the invention.

The core yarn comprising double-threaded-multi-glass filaments has better overall mechanical strength than the core yarn comprising a single filament of glass, due to less strength variation over its length. A second improvement of the core yarn of the third embodiment is better adhesion of the fibers wrapped around the core ply yarn than around the single filament of glass of the core ply yarn of the first embodiment. In addition, the glass filaments used for the core ply yarn of the third embodiment are preferably colored, so that the core yarn is no longer visible through the fibers wrapped around it. Furthermore, because the adhesion of the fibers wrapped around the core ply yarn is better, and the core ply yarn is preferably colored, the warp yarn count need not be 1% to 20% lower than the weft yarn count, as is the case in the second embodiment. To the contrary, the weft yarn count and the warp yarn count are preferably the same. Therefore, only one type of yarn need be spun, which simplifies the weaving of the fabric.

The fire-resistant textile yarn comprising a core formed from a ply yarn comprising double-threaded - multi-glass filaments and the use of this yarn in making clothing fabric is illustrated in detail in the following Examples. These Examples are included for illustrative purposes and should not be considered to limit the present invention.

#### EXAMPLE 1

Yarn of 50 tex, comprising a glass core yarn including double-threaded-multi-glass filaments (2  $\times$  5.5 tex) dyed green by coating produced by the Firm Chavanoz S. A. of the Groupe Porcher, 163 boulevard des Etats-Unis, 69009 Lyon (France). The glass core yarn corresponds to 22% weight of the yarn.

The fibers comprise 50% of Kermel® of Rhone Poulen Textile which is a flame resistant polyamide-imide polymer and 50% of Viscose Flame Retardant; this fiber, which is internally dyed or unbleached, is purchased from the Austrian Firm Lenzing. 70% of the fibers lay parallel to the core yarn and about 30% are wrapped around it.

#### EXAMPLE 2

Yarn of 42 tex, comprising a glass core yarn including double-threaded-multi-glass filament (2  $\times$  5.5 tex) dyed orange by coating, produced by the Firm Chavanoz S. 50 A. The core glass yarn corresponds to 26% weight of the yarn.

The fibers around the core comprise 50% of meta-aramid fibers sold under the registered trademark Connex® of the Japanese Firm TEIJIN, and of Viscose Flame Retardant, as in Example 1. 70% of the fibers lay parallel to the core yarn and about 30% are wrapped around it.

#### EXAMPLE 3

60 Yarn of 55 tex, comprising a glass core yarn as in Example 1. The core yarn corresponds to 20% weight of the yarn.

The fibers around the core comprise 67% of Viscose Flame Retardant as in the preceding Examples and 33% of flame resistant fibers of a copolyimide sold under the trademark P-84 by the Austrian Firm Lenzing. As in the foregoing Examples, about 70% of the fibers lay parallel to the core yarn and about 30% are wrapped around it.

The invention having been described, it will be appreciated by those skilled in the art, that various modifications can be made within the scope of the following claims.

What is claimed is:

1. A fire-resistant textile yarn comprising (1) a core formed from a ply yarn comprising double-threaded-multiple-glass filaments, and (2) fibers wound around the core, wherein at least 33% by weight of said fibers are formed from aramid resin, and the yarn count is between 30-55 tex, the mass ratio of the core is between

10% and 26%, and the fibers are spun without axial twisting around the core.

2. The textile yarn according to claim 1, said fibers around the core comprising 50% aramid fibers and 50% viscose fibers.

3. The textile yarn according to claim 1, said fibers around the core comprising 67% viscose fibers and 33% copolyimide fibers.

4. The textile yarn according to claim 1, said fibers around the core comprising 50% polyamide-imide fibers and 50% viscose fibers.

5. The textile yarn according to claim 1, wherein the glass filaments are colored.

\* \* \* \* \*

15

20

25

30

35

40

45

50

55

60

65